

# UNITED STATES PATENT OFFICE.

PETER THORESON, OF BALDI, WASHINGTON.

## COMPOSITION FOR SHOE DRESSING.

1,415,208.

Specification of Letters Patent. Patented May 9, 1922.

No Drawing.

Application filed May 26, 1921. Serial No. 472,868.

To all whom it may concern:

Be it known that I, PETER THORESON, a citizen of the United States, and a resident of the town of Baldi, county of King, State 5 of Washington, have invented certain new and useful Improvements in Compositions for Shoe Dressing, of which the following is a specification.

This invention relates to improvements in 10 compositions, and more particularly to a composition of matter especially useful as a shoe dressing; the principal object of the invention being to provide a shoe dressing that will resist water, that will act as a preservative to the leather and seams of shoes 15 to which it is applied, and will keep the leather soft and pliable.

A further object of the invention resides in the proper proportioning of the ingredients used and in the manner of mixing the 20 same.

My composition consists of a mixture of pure pine tar, beef tallow, rubber and neat's foot oil.

25 In preparing, I prefer to use the ingredients in about the following measured proportions: one part pure pine tar, one part beef tallow and one part rubber, to which is added one pint of neat's foot oil to each 30 gallon of mixture of the three above ingredients after being reduced by boiling.

The preparation consists of mixing solid 35 texture, beef tallow with rubber, such as used in the inner tubes of automobile tires, and boiling this until it is reduced to a paste.

To this when partly cooled is then added, rendered beef tallow and pine tar that has been warmed so that these ingredients can then be mixed thoroughly. The neat's foot oil is then added in the quantity as above 40 stated, and all are thoroughly mixed and then allowed to cool.

The rubber vehicle provided in the composition, when the latter is applied to the leather of shoes, fills the pores, keeping the 45 leather soft and pliable. The tallow, oil and tar resist water and add to the life of the leather.

Having thus described my invention, what I claim as new therein and desire to 50 secure by Letters-Patent, is:

1. A composition adapted for use as a leather dressing and preservative consisting of a mixture of substantially equal parts, by measurement, of beef tallow, pure pine tar 55 and rubber, to which mixture is added one part of neat's foot oil to eight parts of mixture.

2. The process of preparing a leather dressing from a mixture of beef tallow, pure 60 pine tar, rubber and neat's foot oil, which consists of warming to a liquid and mixing together, the first three ingredients in equal proportions and then adding one pint of neat's foot oil to each gallon of mixture and 65 then allowing the composition to cool.

Signed at Seattle, Washington, this 20th day of May, 1921.

PETER THORESON.